

2,817,628

## ANTIMONY PLATING BATH

Elmer R. Breining, Warren, and William R. Vincent, Birmingham, Mich., assignors to General Motors Corporation, Detroit, Mich., a corporation of Delaware

No Drawing. Application October 16, 1953,  
Serial No. 386,654

4 Claims. (Cl. 204—45)

This invention relates to improvements in the electrodeposition of antimony and more particularly to an improved bath and process for the deposition of smooth adherent coatings of antimony.

In many instances electrodeposits of antimony produced by prior antimony plating solutions and processes have not only been poorly adherent and extremely brittle, but also have exhibited a poor surface quality and have been difficult to buff or polish.

We have now discovered that the aforementioned difficulties can be avoided and improved electrodeposits of antimony obtained from aqueous baths containing sulfonated hydroxy aromatic compounds. Preferred sulfonated hydroxy aromatic compounds contain, in addition to a sulfonate radical and hydroxy grouping on the aromatic nucleus, at least one additional substituted grouping which is capable of complexing dissolved metals to form five or six membered ring systems. Typical of the type of addition agents contemplated in the present invention are the compounds obtained by sulfonating substituted phenols, catechol, derivatives of catechol such as 3-5 dihydroxy toluene (orcinol), isomers of catechol such as resorcinol; trihydroxy phenols such as pyrogallol, phloroglucinol; hydroxy aromatic carboxylic acids such as salicylic acid, B-resorcylic acid; hydroxy aromatic aldehydes such as salicylaldehyde; 8-hydroxy quinoline; and naphthols such as 1-3 or 1-8 dihydroxy naphthalene.

In certain applications, it is advantageous to employ, in addition to or in lieu of the above-mentioned additives, certain unsulfonated compounds including polyhydric alcohols such as glycerol, ethylene glycol, propylene glycol, mannitol, sorbitol, dulcitol, erythritol, or pentaerythritol; unsulfonated sugars such as dextrose, levulose or sucrose; as well as unsulfonated sugar acids such as gluconic, mucic, and saccharic acids. It will be understood, of course, that the present invention contemplates the use of the above addition agents as well as mixtures thereof. Similarly, sodium, potassium, ammonium, amine, or antimony salts of the various compounds may be used.

In general, additives of the present invention form various complex organo-metallic salts which regulate the availability of metallic ions in solution. The actual chemical and electrochemical reactions occurring during plating using the additives of the present invention are not clearly understood at present. However, the following discussion, indicating sulfonated catechol as an additive, is set forth to aid in understanding the invention.

Sulfonated catechols may be used effectively in either acid or alkaline antimony plating baths. It will be understood, of course, that in the sulfonation of catechol, mono, di and tri sulfonic acids are obtained, the amounts of each depending upon the technique of sulfonation. Hence, in the following reactions, although a mono-sulfonic acid is illustrated, similar reactions occur using di-sulfonic acid, tri-sulfonic acid or a mixture of these acids.

The effectiveness of the sulfonated catechol is thought to depend primarily on the complexing of antimonious

hydroxide which, in an acid solution, is indicated as follows:



10 The following reactions indicate the ensuing formation of monosulfonated antimony-catechol complex:



In an alkaline bath a similar series of equilibrium reactions occur as summarized in the following equation:



40 It will be understood, of course, that analogous antimony complexes can be formed using other additives of the present invention. The following table summarizes by compound and corresponding formula some of the antimony complexes formed in accordance with the present invention.

| Compound                      | Formula                                                                                                                                      |
|-------------------------------|----------------------------------------------------------------------------------------------------------------------------------------------|
| 50 Antimony Catechol          | $\text{C}_6\text{H}_3(\text{O}-\text{SbOH})_2$                                                                                               |
| Antimony Pyrogallol           | $\text{C}_6\text{H}_3(\text{O}-\text{SbOH})_3$                                                                                               |
| 55 Antimony Thioglycolic Acid | $\text{SCH}_2\text{COOH}$<br>$\text{Sb} \begin{cases} \diagup \\ \diagdown \end{cases} \text{SCH}_2\text{C=O}$                               |
| 60 Antimony Thiolactic Acid   | $\text{CH}_3$<br>$\text{S}-\text{C}-\text{COOH}$<br>$\text{Sb} \begin{cases} \diagup \\ \diagdown \end{cases} \text{S}-\text{C}-\text{COOH}$ |
| 65 Antimony Thioglycollamide  | $\text{OH}$<br>$\text{CH}_3$<br>$\text{Sb} \begin{cases} \diagup \\ \diagdown \end{cases} \text{S}-\text{C}-\text{CONH}_2$                   |
| Ethylene Glycol               | $\text{C} \begin{cases} \diagup \\ \diagdown \end{cases} \text{Sb}-\text{OH}$<br>linkage                                                     |
| 70 Propylene Glycol           | $\text{C} \begin{cases} \diagup \\ \diagdown \end{cases} \text{Sb}-\text{OH}$<br>linkage                                                     |

| Compound            | Formula                                                                             |
|---------------------|-------------------------------------------------------------------------------------|
| Trimethylene Glycol |    |
| Glycerine           |    |
| Erythritol          |    |
| Pentaerythritol     |    |
| Sorbitol            |    |
| Mannitol            |    |
| Arabitol            |    |
| Dulcitol            |  |

Similar antimony complexes may be formed using polyhydroxy aldehydes and ketones, polyhydric alcohols of the cyclohexane type such as quercitol and inositol, as well as various sugar acids.

In general, organic antimony complexes formed in accordance with the present invention may be characterized as organic esters and/or thioesters having the following structure:



or as



The following is an example of a particular antimony bath of the present invention as used in an acid medium in which the quantities are expressed in grams per liter of solution:

*Example I*

|                     |     |
|---------------------|-----|
| Antimony fluoride   | 220 |
| Sulfonated catechol | 237 |
| Potassium hydroxide | 300 |

The above bath may be used satisfactorily within a pH range from about 1 to 5, the upper pH limit generally being that at which precipitation of antimony or neutralized salts occurs. It is preferred to operate the bath using a current density of from approximately 10 to 25 amperes per square foot. The preferred bath temperature is 120° F. although the bath may be

70  
75

operated at a temperature within the range from room temperature, i. e. approximately 70° F., to about 165° F.

Illustrative of an alkaline bath embodying the invention is the following in which the quantities are expressed 5 in grams per liter of solution:

*Example II*

|                                   |                           |
|-----------------------------------|---------------------------|
| Antimony fluoride                 | 220                       |
| Crude sulfonated catechol mixture | 405 (137 grams catechol). |
| Potassium hydroxide               | 420.                      |

This bath generally may be operated at a pH of 12 or greater over a range of temperatures and at a current density within the range from about 10 to 30 amperes 15 per square foot although at present it is preferred to operate the bath at a temperature of about 140° F. using approximately 12 amperes per square foot.

The following are examples of other antimony plating 20 baths and preferred operating conditions in accordance with the present invention.

*Example III*

|                    |                        |
|--------------------|------------------------|
| Antimony fluoride  | 220 g./l.              |
| Glycerol C. P.     | 92 cc.                 |
| Ammonium hydroxide | To regulate pH to 2.0. |
| Current density    | 25 a. s. f.            |
| Temperature        | 140° F.                |

*Example IV*

|                    |                        |
|--------------------|------------------------|
| Antimony fluoride  | 220 g./l.              |
| Sorbitol           | 160 g./l.              |
| Ammonium hydroxide | To regulate pH to 2.0. |
| Current density    | 20 a. s. f.            |
| Temperature        | 140° F.                |

*Example V*

|                    |                        |
|--------------------|------------------------|
| Antimony fluoride  | 220 g./l.              |
| Mannitol           | 124 g./l.              |
| Ammonium hydroxide | To regulate pH to 2.0. |
| Current density    | 30 a. s. f.            |
| Temperature        | 140° F.                |

*Example VI*

|                    |                        |
|--------------------|------------------------|
| Antimony fluoride  | 220 g./l.              |
| Dextrose           | 75 g./l.               |
| Ammonium hydroxide | To regulate pH to 2.0. |
| Current density    | 25 a. s. f.            |
| Temperature        | 135° F.                |

50

*Example VII*

|                    |                     |
|--------------------|---------------------|
| Antimony fluoride  | 220 g./l.           |
| Sucrose            | 75 g./l.            |
| Ammonium hydroxide | Regulate pH to 2.0. |
| Current density    | 20 a. s. f.         |
| Temperature        | 135° F.             |

55

*Example VIII*

|                    |                     |
|--------------------|---------------------|
| Antimony fluoride  | 220 g./l.           |
| Levulose           | 180 g./l.           |
| Ammonium hydroxide | Regulate to 2.0 pH. |
| Current density    | 20 a. s. f.         |
| Temperature        | 135° F.             |

60

*Example IX*

|                    |                        |
|--------------------|------------------------|
| Antimony fluoride  | 220 g./l.              |
| Mucic acid         | 20 g./l.               |
| Ammonium hydroxide | To regulate pH to 2.0. |
| Current density    | 20 a. s. f.            |
| Temperature        | 125° F.                |

65

*Example X*

|                    |                        |
|--------------------|------------------------|
| Antimony fluoride  | 220 g./l.              |
| Gluconic acid      | 10 g./l.               |
| Ammonium hydroxide | To regulate pH to 3.0. |
| Current density    | 20 a. s. f.            |
| Temperature        | 120° F.                |

## 5

## Example XI

|                                |                              |
|--------------------------------|------------------------------|
| Antimony fluoride              | 220 g./l.                    |
| Catechol sulfonic acid mixture | 125 cc. (75 g./l. catechol). |
| Sorbitol                       | 75 g./l.                     |
| Sodium hydroxide               | To regulate pH to 3.5.       |
| Current density                | 20 a. s. f.                  |
| Temperature                    | 130° F.                      |

## Example XII

|                                |                               |
|--------------------------------|-------------------------------|
| Antimony fluoride              | 220 g./l.                     |
| Catechol sulfonic acid mixture | 190 cc. (114 g./l. catechol). |
| Gluconic acid                  | 50 g./l.                      |
| Sodium hydroxide               | To regulate pH to 4.0.        |
| Current density                | 20 a. s. f.                   |
| Temperature                    | 130° F.                       |

## Example XIII

|                                |                                  |
|--------------------------------|----------------------------------|
| Antimony fluoride              | 220 g./l.                        |
| Catechol sulfonic acid mixture | 200 cc. (120 g./l. as catechol). |
| Levulose                       | 45 g./l.                         |
| Potassium hydroxide            | To regulate pH to 4.0.           |
| Current density                | 20 a. s. f.                      |
| Temperature                    | 125° F.                          |

## Example XIV

|                                |                                  |
|--------------------------------|----------------------------------|
| Antimony fluoride              | 220 g./l.                        |
| Catechol sulfonic acid mixture | 200 cc. (120 g./l. as catechol). |
| Dextrose                       | 45 g./l.                         |
| Potassium hydroxide            | To regulate pH to 3.5.           |
| Current density                | 20 a. s. f.                      |
| Temperature                    | 125° F.                          |

## Example XV

|                     |                         |
|---------------------|-------------------------|
| Antimony fluoride   | 220 g./l.               |
| Sulfonated catechol | 71 g./l. (as catechol). |
| Gluconic acid       | 107 g./l.               |
| Sodium hydroxide    | To regulate pH to 4.0.  |
| Current density     | 24 a. s. f.             |
| Temperature         | 120° F.                 |

## Example XVI

|                     |                          |
|---------------------|--------------------------|
| Antimony fluoride   | 220 g./l.                |
| Sulfonated catechol | 120 g./l. (as catechol). |
| Mucic acid          | 30 g./l.                 |
| Sodium hydroxide    | To regulate pH to 4.0.   |
| Current density     | 24 a. s. f.              |
| Temperature         | 120° F.                  |

It will be understood, of course, that the above examples are illustrative only and that suitable pH adjustments can be made to permit operation in an alkaline medium. Moreover, the particular antimony salts employed, as well as the particular addition agents, may be varied. Although the quantities of bath ingredients can be varied, we have found that in most instances it is desirable to employ one or more compounds of antimony in a sufficient amount to provide from about 20 to 165 grams of metallic antimony per liter of solution and an additive of the present invention in an amount generally within the range of about 20 to 300 grams per liter of solution.

Although the above examples illustrate bath compositions using antimony fluoride, it will be understood, of course, that various antimony salts may be employed such

## 6

as antimony oxide, antimony sulfonate, antimony pentafluoride, antimony pentoxide, potassium meta antomonite, butyl amine antimony tartrate, urea antimony tartrate, aniline antimony tartrate, benzyl amine antimony tartrate, phenyl hydrazine antimony tartrate, ammonium antimony citrate, potassium antimony glycollate, potassium antimony citrate, sodium antimony citrate, antimony potassium tartrate, antimony tartrate and antimony sodium tartrate.

- 10 Similarly, instead of the sodium hydroxide or potassium hydroxide indicated in the examples, the pH may be regulated using ammonia, or organic amines, such as butylamine, trimethylamine or ethanolamine.
- 15 In the electrodeposition of antimony, as in other plating processes, proper preparation of the surface to be coated is essential. In depositing antimony on copper we have found that it is desirable to electrolytically etch the surface to be coated from one to five minutes at about 5 amperes per square foot in a 63% by volume solution of 20 phosphoric acid at room temperature. In depositing antimony on steel it is generally advantageous to etch the steel in nitric acid, preferably diluted 1:3.

25 As an example of the preparation of a plating bath embodying the invention, 890 grams of catechol were added slowly to 1500 grams of C. P. sulfuric acid while maintaining the temperature of the reaction mass within the range from 85° C. to 95° C. for two hours after the last catechol was added. The resultant catechol sulfonic acid-sulfuric acid mixture contained approximately .60 30 gram of catechol per cubic centimeter of crude sulfonation mass. To complete preparation of the bath 241 cc. of the sulfonation mass was then added to an antimony fluoride solution containing 150 grams per liter of metallic ion, the pH adjusted to about 5 using sodium hydroxide, 35 and the resultant mixture heated to 150° F. and treated with activated carbon (3 g./l.) for 2 hours and filtered.

40 It is to be understood that, although the invention has been described with specific reference to particular embodiments thereof, it is not to be so limited since changes and alterations therein may be made which are within the full intended scope of this invention as defined by the appended claims.

What is claimed is:

- 45 1. An electrolytic bath consisting essentially of approximately 20-165 grams per liter of solution of metallic antimony and a complexing agent capable of complexing dissolved antimony to form a five-membered ring, wherein the ring-forming complexing agent is sulfonated catechol present in a concentration of about 20-300 grams per liter 50 of solution.
2. The method of electroplating antimony which comprises passing electric current from an anode to a cathode through the bath of claim 1.
3. An electrolytic bath as in claim 1 in which the antimony is present in the form of antimony fluoride.
4. The method of electroplating antimony which comprises passing electric current from an anode to a cathode through the bath of claim 3.

## 60 References Cited in the file of this patent

- Monthly Review American Electroplaters Society, vol. 29 (1942), p. 870.
- Soderberg et al.: Plating, vol. 37 (1950), pp. 254-259.
- 65 Mathers et al.: Transactions Electrochemical Society, vol. 31 (1917), pp. 293-301.